

## UNITED STATES PATENT OFFICE

1,927,870

## BLACK POWDER COMPOSITION

Benjamin Austin Gillie, Woodbury, N. J., assignor  
to E. I. du Pont de Nemours & Company, Wil-  
mington, Del., a corporation of Delaware

No Drawing. Application March 4, 1930  
Serial No. 433,186

8 Claims. (Cl. 52—17)

This invention relates to a form of explosive of the black powder type, and more particularly to an improved composition of black powder in which the velocity of combustion has been materially decreased.

Black powder is an explosive that has long been known and used, and its general composition over a long period of time has not changed substantially. The usual ingredients entering into its composition are potassium or sodium nitrate, sulfur, and charcoal. Prior to the present invention, a representative composition of black powder has comprised, for example, 72% potassium nitrate, 10% sulfur, and 18% charcoal.

Black powder is generally classified as a low-velocity or deflagrating explosive, as distinguished from the high-velocity, detonating explosives, known as dynamites. This characteristic low velocity of black powder is due to the fact that the black powder contains no ingredient that is explosive in itself, and that an explosive is formed only when an intimate mixture is made of the separate ingredients that are in themselves non-explosive.

Notwithstanding the fact that low velocity is a characteristic of the black powder type of explosives, the different uses of black powder make desirable a control of the velocity that will allow the use of faster or slower powders, as desired.

Various methods have been used heretofore for obtaining increased velocities of combustion.

My invention relates to black powder compositions, and particularly to powders to be used in fuse. For such a purpose, it is desirable that a powder be obtained that will burn at a slow rate, and whose rate of burning is capable of very delicate control. While a slow-burning powder can be obtained by mere adjustment of the percentages of the oxidizing and reducing agents in the black powder, I find such a means unsatisfactory, beyond a certain point. I find a more satisfactory and uniformly slow-burning powder to be obtained, by the introduction into the powder, as an ingredient, of a small percentage of an oil. Various kinds of mineral, animal and vegetable oils may be used for this purpose; for example, various mineral lubricating oils, cotton-seed oil, etc. However, I prefer to use castor oil. While effective amounts of this oil may be introduced, varying considerably in percentage, I find the use of quantities varying from 0.1% to 2.0% by weight to give the desired results, and I preferably use 0.5%. The degree of retardation of the burning speed will depend on the amount of oil used. For example, with very

small percentages of oil, the speed reduction will be slight, while with larger percentages a greater reduction in the speed of burning will be obtained.

Various methods may be used for incorporating the above oil in the black powder mixture. It may, for example, be added directly, by mixing the desired amount with the other ingredients of the black powder under the wheels. Another way of adding the oil to the powder would be to dissolve the oil in a volatile solvent, and then spray the mixture on the powder before final mixing. I prefer, however, to add the oil to the black powder in the form of an emulsion with water. This emulsion may, or may not, contain more than one oil, or may contain some other ingredient for the purpose of further stabilizing the emulsion. Such an emulsion may be added to the other ingredients of the powder and wheeled in with them.

In order to illustrate a specific embodiment of my invention more fully, without in any way limiting the scope of the invention, the following example is given of a fuse powder composition according to my invention:

|                   | Percent |
|-------------------|---------|
| Potassium nitrate | 72.0    |
| Sulfur            | 6.5     |
| Charcoal          | 21.0    |
| Castor oil        | 0.5     |
|                   | 85      |
|                   | 100.0   |

While the above example contains potassium nitrate, it should be understood that this nitrate can be replaced by other nitrates, for example, sodium nitrate, which is the usual oxidizing ingredient in black blasting powder.

The effect of the use of an oil, as described above, in lowering the velocity of combustion of a fuse powder composition is very evident. To determine this delaying effect quantitatively, I find it satisfactory to fill a length of lead fuse with the powder to be tested. This fuse is then rolled down until it has a diameter of approximately 0.15 inches. Under such conditions of testing, I find the time of burning of one foot of my improved powder, containing 0.5% castor oil, to be 57 seconds, against 42 seconds for the same length of fuse powder, of similar composition but containing no speed-reducing oil.

As many apparently widely different embodiments of this invention may be made without departing from the spirit thereof, it is to be understood that I do not limit myself to the fore-

60

65

70

75

80

85

90

95

100

105

110

going examples or descriptions except as indicated in the following patent claims:

I claim:

1. A black powder composition having its rate of combustion retarded by means of an ingredient comprising a solution of a high viscosity, non-drying vegetable oil.
2. A black powder composition having its rate of combustion retarded by means of an ingredient comprising a solution of a non-drying vegetable oil having an absolute viscosity at 40° C. greater than 0.50 dynes per sq. cm.
3. A black powder composition having its rate of combustion retarded by means of an ingredient comprising a solution of castor oil.
4. A black powder composition having its rate of combustion retarded by means of an ingredient comprising an emulsified castor oil.

5. The process of retarding the rate of combustion of a black powder composition which comprises incorporating in the powder a solution of a high viscosity, non-drying vegetable oil.

6. The process of retarding the rate of combustion of a black powder composition which comprises treating the powder with a solution of castor oil.

7. The process of retarding the rate of combustion of a black powder composition which comprises incorporating in the powder and emulsion of a high viscosity, non-drying vegetable oil.

8. The process of retarding the rate of combustion of a black powder composition which comprises treating the powder with emulsified castor oil.

B. AUSTIN GILLIE.

20

95

25

100

30

105

35

110

40

115

45

120

50

125

55

130

60

135

65

140

70

145

75

150